

Oct. 11, 1932.

O. W. STOREY

1,882,046

METHOD OF BLOATING AND ANNEALING BLOCKS OF EARTHY MATERIAL

Filed July 14, 1930

Fig. 1.



Fig. 2.



Witness:

William P. Kilby

Inventor:

Oliver W. Storey  
Donald W. Jamieson

## UNITED STATES PATENT OFFICE

OLIVER W. STOREY, OF MADISON, WISCONSIN, ASSIGNOR, BY MESNE ASSIGNMENTS,  
TO AMERICAN FACE BRICK RESEARCH CORPORATION, A CORPORATION OF ILLINOIS

## METHOD OF BLOATING AND ANNEALING BLOCKS OF EARTHY MATERIAL

Application filed July 14, 1930. Serial No. 467,995.

This invention relates to method of bloating and annealing blocks of earthy material.

In the bloating and annealing of blocks or units of earthy material, difficulty has been experienced by reason of the fact that the blocks or slabs, after being bloated, must be subjected for a considerable period of time to an annealing operation, in order to toughen the bloated material and eliminate strains and stresses therefrom.

Where the material is fed from the bloating chamber and directly through an annealing chamber in a longitudinal direction, this requires an annealing chamber of appreciable length in order to maintain the blocks or slabs of material at the annealing temperature throughout the required period of time.

The method of the present invention is designed to obviate the necessity for a longitudinally extended annealing chamber, by employing a method which results in the stacking up of the blocks or slabs of material in the form of a vertical column which is progressively lowered through a vertically arranged annealing chamber, thereby conserving space in the handling of the material and also serving better to conserve the heat which is retained during the soaking stage of the annealing operation, thereby resulting in a reduction in fuel cost, and in other advantages which will appear from a detailed description of the present invention, in conjunction with the accompanying drawing, wherein,—

Figure 1 is a diagrammatic sectional elevation of the bloating and annealing chambers; and

Fig. 2 is a sectional elevation of the annealing chamber taken on line 2—2 of Figure 1.

The granular material to be bloated is first subjected to a preheating treatment in a rotary kiln 10 at a temperature which will usually run from 1500° F. to 1800° F., and which in all cases should be a temperature slightly below that at which the granular particles begin to fuse and adhere together. After the granular material has been preheated, it is delivered in any suitable manner to a bloating chamber 11 and spread upon the hearth

12 of the bloating chamber (by means which need not be described), in the form of a layer of uniform depth and dimensions.

Thereafter, the layer of material is subjected to a bloating temperature, which causes the granular particles to fuse and coalesce together, and bloat and expand by the formation within the mass of minute cells occasioned by the liberation of gases from within the mass. After the bloating operation has been concluded, and a block or slab of specified dimensions has been produced, the slab is moved rearwardly through an opening 13 in the wall of the bloating chamber and delivered into the soaking and cooling section of the furnace, which as shown comprises a well or pit 14 of suitable depth to permit the bloated slabs to be subjected to a soaking temperature throughout a sufficiently prolonged period of time to eliminate strains or stresses and toughen the material in preparation for the gradual cooling operation.

For certain clays from central and eastern Illinois, the bloating zone will be maintained at a temperature of approximately 2200° F., while the soaking temperature will be maintained at approximately 2000° F. to 2050° F., which is a temperature intermediate the bloating temperature and the congealing temperature, so that during the soaking stage of the operations, the blocks of material, while still in a slightly plastic condition, will become annealed and toughened by the elimination of internal strains or stresses before the temperature is reduced to the congealing point. The temperatures given serve merely as an illustrative example and may be varied as conditions require.

The well or pit 14 may be of sufficient depth to allow the slabs to be first soaked for a sufficient length of time and thereafter cooled during the final stages of their descent through the pit, or if desired the pit can be of sufficient depth only to provide for the soaking operation and cooling to the congealing point, and the slabs can be afterwards removed from the base of the pit and afterwards gradually cooled in any suitable manner. As the slabs are delivered to the pit, they may be progressively lowered in any

suitable manner, as for instance by the provision of vertically movable pairs of fingers 15, 16 and 17, which as shown are arranged in series and are adapted to be thrust inwardly to engage the slabs as they are successively discharged from the bloating chamber into the annealing pit.

In arranging for the descent of the first slab of bloated material, a temporary platform or plunger may be moved upwardly in position to engage the slab as it is shoved inwardly along the hearth, and thereafter the first slab will be lowered sufficiently to bring its upper surface into flush relationship with the hearth. The next slab of material, after bloating, will be moved inwardly by any suitable means, such as a pusher rod 18, until it rests upon the first slab, and thus a column of slabs will be formed and progressively lowered until the fingers are reached, after which the platform or plunger may be dispensed with.

As the column descends in close proximity to the bottom of the pit, the fingers 15 will be moved inwardly to engage the slab next above the lowermost slab, thus temporarily supporting the column from the fingers 15, after which the lowermost slab resting on the fingers 16 may be moved downwardly from the column and deposited upon the lowermost fingers 17 in preparation for a further lowering, which ultimately deposits the slab upon the rails 11 in preparation for its removal by the action of a pusher rod 19 operating through an aperture 20 in the base of the pit.

The fingers may be easily inserted beneath the edges of the respective blocks or sections, by reason of the fact that in bloating, each block or section will assume a rounding edge configuration, which when the slabs are stacked up in column form will afford in each instance an underlying groove or channel into which the fingers may be inserted to the extent required to afford support for the overlying column.

It will, of course, be understood that the use of fingers or the like serves merely for purposes of illustration, and that any other suitable or convenient means may be employed for progressively lowering a column of slabs through the annealing pit by successive stages as the oncoming bloated slabs are delivered at the top of the column.

By stacking the slabs in flatwise relation upon one another, the heat imparted during the bloating operation will be largely conserved and utilized during the soaking operation, although, if necessary, additional external heat may be imparted to the slabs while in the soaking zone, in order to maintain a soaking temperature above the congealing point during the period of time required for the soaking operation.

As before stated, a soaking temperature

may be maintained in the upper portion of the pit, which will thus constitute the soaking zone, while the lower portion of the pit may be maintained at a progressively cooling temperature, so that in such case the pit will combine the function of a soaking zone and a cooling zone, and ultimately deliver the blocks in a sufficiently cooled condition to permit of their being easily handled or transported.

The vertical arrangement of the pit is one which adapts it readily to the maintenance of varying temperatures, since a soaking zone of higher temperature may be readily maintained at the top of the pit by the natural upflow of heated air, while a progressively cooling temperature may be readily maintained at successive stages in the descent of the material through the pit.

The method of the present invention is one which enables the slabs or blocks of material to be easily handled within a relatively small compass and obviates the necessity for the utilization of large areas of floor space for the accommodation of elongated soaking and cooling chambers.

I claim:

1. The method of bloating and annealing blocks of earthy material, which consists in subjecting a charge of granular material to a bloating temperature maintained in an elevated bloating zone to form a unit slab of bloated material, laterally moving the bloated slab away from the bloating zone to an annealing zone, and lowering the slab through the annealing zone, and in superposing successive slabs in column form for movement through the annealing zone.

2. The method of bloating and annealing blocks of earthy material, which consists in subjecting a charge of granular material to a bloating temperature maintained in an elevated bloating zone to form a unit slab of bloated material, laterally moving the bloated slab away from the bloating zone to an annealing zone, and lowering the slab through the annealing zone, and in superposing successive slabs in column form for movement through the annealing zone, and in successively lowering the lowermost slabs of the column below and away from the column and removing them from the annealing zone.

3. The method of bloating and annealing blocks of earthy material, which consists in successively depositing unit layers of earthy material within a bloating zone and subjecting them to a bloating temperature to cause fusion of the particles, and bloating and expansion in the formation of a block of cellular material, successively discharging the blocks by lateral movement from the bloating zone to a vertically extending annealing zone, and progressively forming a column of blocks within the annealing zone, and progressively lowering the column and in main-

taining the upper portion of the annealing zone at a soaking temperature, and the lower portion of the annealing zone at a progressively cooling temperature.

4. The method of bloating and annealing blocks of earthy material, which consists in successively depositing unit layers of earthy material within a bloating zone and subjecting them to a bloating temperature to cause fusion of the particles, and bloating and expansion in the formation of a block of cellular material, successively discharging the blocks by lateral movement from the bloating zone to a vertically extending annealing zone, and progressively forming a column of blocks within the annealing zone, and progressively lowering the column and in maintaining the upper portion of the annealing zone at a soaking temperature, and the lower portion of the annealing zone at a progressively cooling temperature, and in successively releasing the lowermost blocks from the column after the descent through the annealing zone, and laterally transporting the released blocks.

25 In witness that I claim the foregoing I have hereunto subscribed my name this 30th day of June, 1930.

OLIVER W. STOREY.

20

35

40

45

50

55

60